

May 7, 1940.

C. B. WHITE

2,200,139

## PROCESS FOR RECOVERY OF METALS FROM ALLOYS AND METALLURGICAL RESIDUES

Filed Feb. 1, 1939



Clarence B. White

Eugene C. Brown

Attorney

## UNITED STATES PATENT OFFICE

2,200,139

PROCESS FOR RECOVERY OF METALS FROM  
ALLOYS AND METALLURGICAL RESIDUES

Clarence B. White, Philadelphia, Pa.

Application February 1, 1939, Serial No. 254,123

1 Claim. (Cl. 204—15)

This invention relates to the separation of metals from scrap material, metallurgical by-products and commercial residues containing copper, lead, tin, zinc, iron, nickel, antimony, 5 silver, etc., and the recovery of electrolytic copper and lead.

One of the objects of my invention is to provide a method of obtaining pure copper electrolytically from a foul solution containing substantial quantities of zinc, nickel, iron, etc. Another object is to recover and regenerate the spent electrolyte in order to provide a continuous cyclic process. These and other objects will appear 10 from the following description taken in connection with the accompanying drawing which is a schematic illustration of apparatus for practicing my process.

The brass, bronze and other alloy materials may be first reduced in a blast or smelting furnace to separate the metals from the non-metallic 20 contents and the molten metal is then cast directly into the form of anode plates suitable for deposition in the electrolytic tanks.

The cast alloy anodes A with a corresponding 25 number of thin sheet copper cathodes C, are suspended in a tank 1, containing an electrolyte of an acid solution of copper nitrate. The copper nitrate is derived by passing a spray of nitric acid through a mass of copper scrap or shot 30 in leaching tower 6, the electrolyte being first heated in a container 7.

Under favorable conditions the copper, lead, 35 iron, nickel and most of the zinc dissolve in the acid electrolyte; while the tin, antimony, silver and a portion of the zinc, do not go into solution but form a sludge, which either adheres to the anodes or settles to the bottom of the tank and is cleaned off periodically.

As is well known successful electrolysis is dependent upon a constant supply of ions at the 40 cathode. When a soluble anode is employed, ions are supplied at the anode by the solution of the copper and thereby very greatly reduces the voltage required to plate the copper upon 45 the cathode. Best results are obtained with a current of from .20 to .30 volts per plate and a current density of from 12 to 18 amperes per square foot of cathode surface although satisfactory results may be obtained with other current 50 densities. Moreover the continuous replenishment of the copper nitrate by the dissolving copper does not interfere with the efficient operation of the electrolytic action, whereas when a copper sulphate electrolyte is employed, the solution in 55 the immediate vicinity of the anode is always

supersaturated as the copper dissolves and copper sulphate will crystallize on the electrode if the acid content is too high, thereby rendering the anode less soluble, with the consequent cutting down of the copper content of the electrolyte and an increase in the voltage required.

Under proper conditions I obtain copper cathodes of 99.97 to 99.99 per cent purity. Favorable conditions exist with an electrolyte of acidity registered by pH from 1 to 2 at a temperature of 40° to 55° C., with a content of 30 to 40 grams of copper per liter and an electrolyte circulation of 4 gallons per tank per minute. Other combinations of temperature, acidity and copper content can be employed satisfactorily. 15

When the lead content of the electrolyte in tank 1 builds up to a worthwhile concentration, as for example, from 10 to 15 grams per liter, the solution is allowed to pass into a tank 2, which is provided with thin sheet copper cathodes C' and insoluble anodes I, such as platinum, carbon etc. By electrolytic action in this tank, the lead is recovered at the anode as pure lead peroxide PbO<sub>2</sub>, while copper from the electrolyte is deposited upon the cathode with some regeneration of acid. The electrolytic solution is then pumped from tank 2 to the spray head 10 of the uppermost section of the condenser 12.

When the solution in tank 1 builds up with zinc, nickel, iron and other impurities to an extent that might interfere with the efficiency of the electrolytic process, it is transferred to tank 3 having insoluble anodes I and thin sheet copper cathodes C<sup>2</sup>, in which the lead and copper content are completely removed electrolytically. The 35 resulting solution is transferred to a still 14 in which it is heated to break up the nitrates. The nitric acid together with any oxides of nitrogen are collected in the condenser 12. The residue contains oxides of zinc, nickel, iron, etc. which 40 can be treated by the usual metallurgical processes to recover the zinc and nickel.

The oxides of nitrogen from the evaporator 14 together with the oxides of nitrogen and air supply from the leaching tower 6 pass into the lowest scrubbing section of the condenser 12 and percolate upwardly through the mass of broken stone 13 or other suitable rubble inert to nitric acid, such as quartz, rock or chemical stoneware, to combine with the spent electrolyte 50 entering through the spray heads 10 in the upper part of each condenser section and thereby regenerate the supply of nitric acid.

The recycling of the spent electrolyte in countercurrent relationship to the flow of the gaseous

oxides of nitrogen, provides a continuous cyclic renewal of the nitric acid solvent. This feature of the method is of great importance and is a vital factor in the practical recovery of metals from scrap metal and metallurgical by-products by means of nitric acid solvents on a commercial scale.

By the process disclosed herein, copper of the highest purity may be obtained electrolytically, 10 directly from unrefined commercial scrap metal and is deposited from a foul electrolyte. Whereas the quality of the electrolytic copper produced by the leading refineries runs about 99.96% pure, I am enabled to obtain copper of 99.97 to 99.99 15 per cent purity by the process described herein. It will be appreciated by metallurgists that this small improvement in quality is important. Furthermore spectrographic tests of copper obtained by my method show less and fewer impurities 20 than electrolytic copper made by the sulphate process. Also, as pointed out above, my present process requires less current to maintain a con-

stant supply of ions at the cathode during the electrolytic process.

I claim:

The method of treating materials such as scrap metal, brass, commercial residues and metallurgical by-products, containing copper in major amount and metals such as, tin, lead, zinc, nickel and silver in minor amount to separate and recover said individual metals, which comprises melting said materials and casting the molten metal into the form of anodes, utilizing said anodes with cathodes of copper or other suitable material in an electrolyzing tank containing an electrolyte consisting essentially of a nitric acid solution of copper nitrate passing an electric current between the anodes and cathodes to dissolve the copper, lead, zinc, iron and nickel from the anodes, the tin and silver separating from the anodes as a sludge, and to deposit only substantially pure copper upon said cathodes. 20

CLARENCE B. WHITE.